

No. 669,750.

Patented Mar. 12, 1901.

D. B. JONES.

METHOD OF MAKING ZINC WHITE.

(Application filed July 14, 1899.)

(No Model.)

Fig. 1.



Fig. 2.



Witnessed:  
Oliver D. Dennis,  
Alberta Adamick

Inventor:  
David B. Jones  
By Brian T. Fisher  
Atty. Attorney.

# UNITED STATES PATENT OFFICE.

DAVID B. JONES, OF CHICAGO, ILLINOIS.

## METHOD OF MAKING ZINC-WHITE.

SPECIFICATION forming part of Letters Patent No. 669,750, dated March 12, 1901.

Application filed July 14, 1899. Serial No. 723,773. (No specimens.)

*To all whom it may concern:*

Be it known that I, DAVID B. JONES, of Chicago, Illinois, have invented certain new and useful Improvements in Methods of Making Zinc-White, of which the following is hereby declared to be a full, clear, and exact description.

In usual practice zinc-white is ordinarily obtained by subjecting the broken ore and fuel admixed with a minor quantity of flux to the action of an air-blast, the charge resting upon the grate-bars of the familiar Wetherell furnace. High-grade ores containing fifty per cent. or more of zinc are usually selected not only because of the relative cheapness of furnace management due to excess yield, but also by reason of the freedom of the ore from any large percentage of iron or other deleterious ingredient. The heat developed effects reduction of the iron, which thereupon fluxes and disappears in the slag. If the iron be excessive, the slag becomes more copious and tends to unite the charge as a matte on the fire-bars of the furnace. Besides, the slag acts as a barrier to the free distillation of the zinc, so that a considerable quantity is detained in the refuse gangue and becomes lost.

The object of the present invention is to accomplish the economic utilization of zinc-ores of low grade for manufacture of zinc-white despite the marked percentage of iron, &c., (e. g., manganese,) with which the zinc-ores are generally contaminated. Ores containing twenty-five per cent. zinc, for example, often carry an equal or even higher content of iron, both elements being combined with sulfur to constitute a poor zinc-blende or "black jack" of commerce.

In practice the selected ore is finely comminuted or powdered and admixed with an equal or even greater quantity of fuel sufficient to support desired combustion. In conjunction with a minor addition of usual flux, similarly reduced, the powdered mixture is projected as a charge in divided masses by aid of an air-blast into the interior of an upright furnace. The direction of the blast is substantially tangential, so that the charge assumes a swirling or cyclonic motion within the furnace, while the fuel, emerging in divided masses separate from each other, bursts

into flame and effects rapid reduction and conversion of the volatile zinc. The pigment-fumes escape at the furnace-throat into the familiar collecting-chambers. The high heat and the swirling motion effect the separation of the iron and other non-volatile constituents from the zinc, these for the most part becoming slagged and on contact with the furnace-walls falling away thereon to the pit beneath. A bright fire at the pit serves to start the furnace in action, but later on may be diminished or be even dispensed with, except so far as may be requisite to keep the slag melted for occasional tapping.

On the accompanying drawings, Figure 1 is a longitudinal and Fig. 2 a cross-section view of one style of furnace properly suited for practice of the invention.

As here shown, the furnace-body A is of taper or hopper like form, ending below in a slag-pit B and surmounted by a dome-top C, having escape-pipe D for discharge of the pigment-fumes into the collecting-chambers. A chute E admits fuel to the pit B, and an ordinary bustle-pipe F, with twyvers f, distributes the air-blast for the subsidiary fire. At some distance above the contracted base or pit delivery-pipes G project tangentially through the furnace-wall and by aid of an air-blast serve to feed the mixed charge of ore, fuel, and flux in divided masses at separate points within the furnace, a swirling motion being imparted to the charge by reason of the direction of delivery and the encounter with the furnace interior. The taper wall is of advantage, affording easy expansion for the combustion products toward the exit and ready clearance for the pigment-fumes from the associated non-volatile constituents. Any suitable mechanism can be employed for supplying the powdered charge as a burden to be floated in the air-blast on its way to the furnace. Owing to the mode of delivery and the copious volume of air and fuel supplies the combustion becomes intense, the sulfur rapidly burns away, leaving the zinc free to reduce and convert into pigment-fumes, while the iron fuses in the flux and during its swirling progress separates as a slag on contact with the furnace-wall.

Obviously the details of structure can be varied according to the mechanic's skill without departure from the invention.

Having thus described my invention, what I claim as new, and desire to secure by Letters Patent, is—

The method of making zinc-white which consists in imparting a cyclonic swirl to the admixed charge of powdered ore, fuel and flux by projecting it tangentially in divided masses through aid of an air-blast into the

furnace, setting the charge afame, expanding the resultant pigment-fumes and combustion products freely upward toward the exit and simultaneously separating and trapping the associated non-volatile constituents or slags by arrest thereof during the centrifugal swirl, substantially as described. 15

DAVID B. JONES.

Witnesses:

GEO. P. FISHER, Jr.,  
ALBERTA ADAMICK.